

Nov. 4, 1947.

K. A. SPENCER ET AL

2,430,085

PROCESS OF PREPARING COAL FOR USE IN COLLOIDAL FUELS

Filed July 9, 1943



## UNITED STATES PATENT OFFICE

2,430,085

PROCESS OF PREPARING COAL FOR USE IN  
COLLOIDAL FUELS

**Kenneth A. Spencer, Kansas City, and Donald W. Machin, Lawrence, Kans., assignors to The Pittsburg and Midway Coal Mining Company, Pittsburg, Kans., a corporation of Missouri**

Application July 9, 1943, Serial No. 494,006

1 Claim. (Cl. 241—17)

**I**

This invention is concerned with a process of preparing coal for use in composite coal-oil fuels commonly referred to as colloidal fuels.

Examples of prior art processes may be found in the U. S. patents to L. W. Bates, No. 1,390,228; C. J. Greenstreet, Nos. 1,431,225 and 1,623,241; H. Plauson, No. 1,647,471; R. A. Adam, No. 1,939,587; and A. L. Stillman, No. 2,231,513.

The new process comprises the following principal steps: First, the step of far-reaching dehydration of previously de-ashed, i. e., washed lump size coal prior to pulverization thereof; second, the step of withdrawing coal fines incident to dehydration and collecting such fines for use and intermixture with a suitable fuel oil; third, pulverization of the dehydrated lump size coal in two separate and distinct operations; fourth, separation of the pulverized coal which furnishes in the form of undersize a selected product suitable for dispersion in the fuel oil and in the form of oversize a product which is re-circulated through the pulverizing apparatus; and fifth, uniting the coal fines extracted from the feed incident to dehydration with the selection fines obtained by the separation of the pulverized coal, and dispersing such fines in a suitable fuel oil.

The combination of these steps, and particularly the dehydration of the coal and the steps of feeding to the pulverizing and thence to the separating apparatus the previously dehydrated coal are important features which have a profound effect on the all-important question of economy of producing the colloidal fuel. The dehydration of the coal also aids the proper dispersion of the particles in the oil and thereby benefits the stability of the final product.

The new process is described below in detail with reference to the accompanying single sheet of drawings showing in diagrammatic manner the organization and coaction of apparatus for processing the coal and also showing, for the sake of completeness, the principal apparatus for dispersing the processed coal in a suitable fuel oil.

The equipment used in the process is well known and the principal units are diagrammatically indicated. Auxiliary apparatus, such as conveyors, elevators, feed belts, drives, various control means, and the like are omitted.

Washed, i. e., previously de-ashed, bituminous coal of a maximum lump size of about  $\frac{3}{4}$  in.

is fed to the drum 11 of a suitable heat drier. This drier may be of the rotary type as indicated in the drawing. The coal flows through the drier in the direction indicated by the arrow, and is subjected to an air current, sweeping through the drum, which has been heated to a mean temperature of about 350° F. in a furnace 12. The feed of the coal and the speed of rotation of the drum are adjusted so as to subject the coal to the action of the heated air current for a time sufficient to effect substantially complete removal of moisture, i. e., to a point when the moisture content is reduced to less than 1%.

The step of dehydrating coal of substantial lump size, as indicated, permits the application of higher temperatures, and longer treatment times than could be applied with safety if the material were ground to appreciably smaller size. It may be mentioned at this point that we applied appreciably higher temperatures, up to 500° F., for short periods of time, without any ill effect. The mean temperature was, however, as stated, 350° F. The process of removing the moisture is accelerated by this mode of operation, and the danger of combustion is eliminated. The treatment can be applied with available equipment of proved performance.

Air containing coal fines is withdrawn from the heat drier, by a suction fan 13, and is conducted into a dust precipitation chamber 14. These coal fines are on the order of about 200 mesh, suitable for dispersion in the oil. They are collected and either supplied to a sacker bin 21, for storage, or to a feeder device 20 for mixing with the oil.

The step of removing coal fines from the heat drier, as described, serves a double purpose. It contributes to the safety of the moisture removal operation within the drier, and results in saving appreciable amounts of material for dispersion in the oil.

The moisture-free lump coal flows from the heat drier 11 into and through the cooler 15 to reduce its temperature to around 100° F. The cooler may be of the rotary type and may form part of the drier unit as shown. The material is then directed to a crusher 16 which performs the first pulverizing operation by reducing the lump size to about  $\frac{1}{4}$  in. Any suitable crusher may be used for this purpose.

**2**

## 3

The operation of the crusher is accelerated and is rendered economical by the dry condition of the material which is still at elevated temperature.

The 0 by  $\frac{1}{4}$  in. dehydrated coal is then fed to a suitable mill 17 which performs the second and final pulverizing operation by reducing the coal to a particle size of about 200 mesh. Any suitable mill may be used; the mill actually employed was a ball mill of well known structure.

The step of feeding substantially moisture-free material at elevated temperature to the mill 17 accelerates the final pulverizing operation and therefore contributes to the economy of the process. The pre-grinding of the lump size coal to a particle size of about  $\frac{1}{4}$  in. has been found best for the efficient operation of the pulverizing mill.

The dry pulverized material coming from the mill 17 is fed to an air separator 18 commonly referred to as a cyclone. This separator delivers two products, namely, the product of desired particle size of about 85% to 95% through 200 mesh, which is either supplied to a sacker bin 19 for storage, or to the feeder device 20 for dispersion in the oil, and an oversize product which is recirculated through the pulverizer mill 17.

The step of feeding substantially moisture-free material to the cyclone separator accelerates and renders more accurate the sizing operation, resulting in a greater yield of selected fines per time unit, thereby adding to the economy of the process.

The discharge into the sacker bins 19 and 21 (a single bin may be used for receiving material from the separator 18 and also from the dust precipitator 14) is practiced when it is desired to prepare coal for temporary storage and subsequent dispersion in the oil. The sacker bin is an ordinary bin or hopper which receives the pulverized material for discharge into storage sacks provided with moistureproof lining.

The process may also be continuous, and in this case, the pulverized material from the precipitator 14 and from the separator 18 is collected in a suitable bin (not shown) and is then fed in measured, controlled amounts to the mixer 22, during the mixing operation, by means of the feeder 20. The latter may be an ordinary screw feeding device, as indicated. Its speed controls the amount of coal fines gradually supplied to the mixer.

The mixer 22 may be equipped with a propeller or a plurality of propellers, according to its size and the desired speed of processing. Heating coils may be provided within the mixer tank and supplied with steam in order to carry out the mixing at elevated temperatures between 150° F. and 200° F.

Oil is supplied from the reservoir 23. Coal is gradually added, during mixing, in an amount to provide a final mix containing about 40% of coal by weight. Samples are taken during the initial mixing operation, and subjected to tests, so as to determine the proper dispersion of the coal particles in the oil and therewith the optimum mixing time for subsequent operation. The finished fuel is withdrawn from the tank 22 for storage or use.

A colloid mill 24 may be used in place of the mixer 22, or may receive a rough mix, produced in the mixer 22 at a shorter mixing time, for homogenizing. Such operation is well known and need not be described in detail. The finished product is then withdrawn from the colloid mill for storage or use.

The coal actually used in the above described

75

## 4

process was washed bituminous Kansas coal. It is, of course, clear that other coal, and various combustible solids, such as are mentioned in the prior art patents, may be employed equally well. The process was practiced with numerous kinds of fuel oils. Production was successfully carried out, using 6.0 A. P. I. residual fuel oil with a Saybolt Furol viscosity of 220 sec. No stabilizer was used and none appears to be required in this case. The fuel remained stable in testing, in storage, during transport in tank cars, and during large scale industrial combustion tests ordinary equipment provided for oil burning.

The process disclosed herein is not restricted to the use of heavy fuel oils such as mentioned. The combustible solids, prepared as described, may also be dispersed in lighter combustible liquids. Stabilizers may be employed if desired or required.

The far-reaching, substantially complete removal of moisture benefits not only the economy of production, as previously explained; it is also believed to aid the dispersion of the coal particles in the oil and therewith to benefit the stabilization of the final product. This will be understood when it is considered that coal containing moisture presents surfaces to the oil which are moist and, therefore, lyophobic with respect to the oil. This means that these surfaces are liquid-repellent, producing a system in which the dispersed phase has no attraction for the dispersion medium and therefore tends to separate. Coal that is practically completely dehydrated, such as is used in the present process will, on the other hand, assist lyosorption, i. e., the adhesion of the liquid to the solids, and will therefore tend to produce adsorption of solvent films upon the surfaces of the particles dispersed and suspended in the oil. It is believed that the dehydration of the coal, as previously described, accounts in part for the stability of the colloidal fuel produced.

Changes may be made within the scope and spirit of the following claim in which is pointed out what is considered new and desired to have protected by Letters Patent of the United States.

We claim:

The process of preparing coal for use in colloidal fuels which consists of the following steps, in the sequence specified, namely, (1) taking lump size de-ashed bituminous coal within a size range from 0" to about  $\frac{3}{4}$ " and dehydrating such coal to a moisture content of less than 1% in the presence of heat ranging from about 350° F. to about 500° F.; (2) withdrawing during such dehydration fines which are about 200 mesh; (3) cooling the dehydrated coal to a temperature of about 100° F.; (4) pre-crushing the dehydrated and cooled coal at a temperature of about 100° F. retained therein to obtain particles of a size range from 0" to about  $\frac{1}{4}$ "; (5) pulverizing the pre-crushed coal at a temperature of about 100° F. retained therein to obtain a product of about 85% to 95% through 200 mesh; (6) separating from the pulverized product particles of about 200 mesh; and (7) intermixing the separated particles of about 200 mesh with the fines of about 200 mesh withdrawn during the dehydration of the lump size coal.

KENNETH A. SPENCER.  
DONALD W. MACHIN.

(References on following page)

## REFERENCES CITED

The following references are of record in the file of this patent:

## UNITED STATES PATENTS

| Number    | Name       | Date          | Number    | Name      | Date          |               |
|-----------|------------|---------------|-----------|-----------|---------------|---------------|
| 1,390,231 | Bates      | Sept. 6, 1921 | 2,175,484 | Rees      | Oct. 10, 1939 |               |
| 2,029,917 | Frisch     | Feb. 4, 1936  | 2,319,394 | Erickson  | May 18, 1943  |               |
| 1,977,501 | Townsend   | Oct. 16, 1934 | 1,491,841 | Bell      | Apr. 29, 1924 |               |
| 1,390,228 | Bates      | Sept. 6, 1921 | 5         | 1,710,666 | Newhouse      | Apr. 23, 1924 |
| 1,939,587 | Adam       | Dec. 12, 1933 |           |           |               |               |
| 2,231,513 | Stillman   | Feb. 11, 1941 | 410,883   |           |               |               |
| 1,458,106 | McLaughlin | June 5, 1923  |           |           |               |               |
| 1,991,583 | Stockton   | Feb. 19, 1935 | 10        |           |               |               |
|           |            |               | 15        |           |               |               |

| Name     | Date          |
|----------|---------------|
| Rees     | Oct. 10, 1939 |
| Erickson | May 18, 1943  |
| Bell     | Apr. 29, 1924 |
| Newhouse | Apr. 23, 1924 |

## FOREIGN PATENTS

| Country       | Date         |
|---------------|--------------|
| Great Britain | May 31, 1934 |

## OTHER REFERENCES

Pulverizing 200 Process Materials, pages 241-2 of Chemical and Metallurgical Engineering, volume 45, No. 5, May 1938. McGraw Hill Book Company, New York. (Copy in 241-30.)